

March 16, 1926.

1,576,883

V. M. WEAVER

PROCESS OF MAKING GRAPHITE

Filed March 2, 1923



FIG. 1



FIG. 2

Inventor

Victor M. Weaver

By

Lloyd L. Evans

Attorney

## UNITED STATES PATENT OFFICE.

VICTOR M. WEAVER, OF HARRISBURG, PENNSYLVANIA.

## PROCESS OF MAKING GRAPHITE.

Application filed March 2, 1923. Serial No. 622,298.

*To all whom it may concern:*

Be it known that I, VICTOR M. WEAVER, a citizen of the United States, and a resident of Harrisburg, county of Dauphin, 5 State of Pennsylvania, have invented a certain new and useful Improvement in Processes of Making Graphite, of which the following is a full, clear, and exact description, reference being had to the accompanying drawings.

This invention relates to the art of manufacturing relatively dense or crystalline forms of carbon from carbonaceous material.

More particularly it has for its object 15 the manufacture of graphite and especially dense forms thereof.

An object of this invention is to make graphite slabs suitable for electrodes which are of uniform, relatively dense, homogeneous character and which will be suitable 20 for use in the electrochemical or other arts wherever such characteristics are desirable.

A further object of this invention is to produce such graphite in relatively large 25 quantities and in a relatively cheap manner and of a predetermined form so that it can be used, if desired, as an electrode without additional cutting and shaping.

Another object of the invention is to produce graphite without the use of the customary pitch binder or the like, which in heating volatilizes and causes the electrode to become relatively porous.

A further object of this invention is to 35 virtually cast carbonaceous material into graphitic slabs or ingots by the use of a flux capable of flowing the material and of being broken down to leave graphite.

Another object of my invention is to produce graphite shapes or slabs which can be mechanically pressed or worked while the slab is hot to force the particles relatively close together and thereby produce a more dense slab of crystalline carbon.

45 According to the usual methods of manufacturing graphite slabs or electrodes the carbonaceous material is first calcined and then ground and pulverized. This pulverized material is then mixed with a binder, 50 such as a pitch binder. This material is then pressed or extruded into the desired shapes and heated usually in an electric furnace. To obtain graphite the temperature must be relatively much higher than for

the so-called carbon electrodes. During the 55 final baking a relatively large part of the binder is volatilized and driven off and this naturally leaves the electrode more or less porous. Thus it will be seen that the shaping and manufacture of carbon or graphite 60 electrodes has been analogous, generally, to the methods of operation in the ceramic industry. That is, carbon has been treated as an infusible substance and all of the working of the material and the application 65 of pressure in the forming steps is performed before the material is finally baked.

As distinguished from these methods of operation and the analogy to ceramics, I 70 have made observations which show that 70 carbonaceous material, such as graphite, can be treated in a manner analogous to metals, and by such treatment can be made, worked, and formed to produce relatively cheaply 75 uniform, relatively dense, homogenous, slabs 75 or ingots of graphite.

I have observed that at relatively high 80 heats carbonaceous material is somewhat plastic and that under certain conditions and with certain fluxes such material can 80 be transformed into graphite and can be made to flow. According to my process, 85 therefore, I select a flux which has the property of transforming carbonaceous material into graphite and which will flow at relatively 85 high temperatures in the presence of graphite and which finally upon reaching a higher temperature will break up into volatile matter leaving graphite. The volatile 90 matter combines with the carbonaceous material above, forming more of the flux. Such a flux, for example, is calcium carbide. This flux has the property of becoming relatively thin and fluid at high 90 temperatures with graphite present, and upon further heating the calcium will be volatilized, leaving the carbon previously combined in the calcium carbide as graphite.

The volatile calcium driven off by this 95 reaction combines with more of the carbonaceous material to form more calcium carbide. These reactions continue progressively until all of the carbonaceous material is 100 transformed into graphite. By utilizing the properties of calcium carbide or an 100 equivalent flux which becomes relatively thin and fluid at high temperatures, I am 105 enabled to flow the carbonaceous material

in the furnace, so that when the operation is complete a relatively dense slab or ingot of graphite of the same shape as the containing walls thereof will be left in the furnace.

- It has also been my observation that carbonaceous material at a relatively high heat softens and becomes pasty and somewhat coalescent. This property I utilize to make 10 the previous slabs of graphite more dense than they would be if simply allowed to cool after formation according to the process herein described. This is accomplished by working or pressing the graphite slab 15 while it is sufficiently hot to be somewhat soft and plastic, that is, while it is above a red heat. It may be done by transferring the slab from the electric furnace in which it is formed to a mold of suitable material 20 and exerting a pressure as with a plunger of a press for a very short period of time and then removing the slab from the mold. Or the furnace itself, if suitably designed, may be used as the die to hold the ingot during 25 the application of pressure. Under certain conditions, if the pressing be done relatively quickly, metal dies, preferably lined with a suitable protective coating of refractory material, may be used, as the heat 30 received by them would be conducted through the relatively large mass of metal sufficiently rapidly to prevent the destruction of the die before the graphite slab can be pressed and removed from the die. 35 By subjecting these graphite slabs to this temperature and pressure treatment, the density of the carbonaceous material can be raised very materially and in fact it seems that under proper conditions the density can be raised to 3.5, or that of the diamond.

In the accompanying drawing wherein I have shown for illustrative purposes an electric furnace for carrying out my process,

40 Figure 1 is a longitudinal sectional view through the furnace.

Fig. 2 is a transverse section through the furnace.

45 In carrying out my process I use a trough-shaped furnace 1, having retaining walls of any suitable material, preferably iron. The bottom and side walls of the furnace are lined with a suitable heat insulator 3, such as powdered carbon or graphite, preferably lamp black. Resting on this lining are 50 slabs of carbon 2, forming the bottom of the inside of the furnace.

A vertically movable frame 4 rests on the 55 carbon floor 2 around its periphery until the furnace has been charged and is ready for operation. Before the furnace is started the frame is raised slightly above the floor and is gradually moved upwardly as the ingot forms. The carbonaceous material from the charge constantly falls between the

ingot and the moving frame and keeps the frame from being destroyed by the heat. The movable frame 4 prevents the lining of heat insulating material 3 from falling into the furnace during the heating operation and, by thus preserving the lining walls intact, insures that the ingot will be of the shape desired. Under certain conditions, if desired, the walls 4 may be of carbon and left in place during the heating.

Any number of electrodes 5 suitable to heat the contents of the furnace may be used. These electrodes are preferably located so as to draw arcs from the surface of the bottom 2 of the furnace proper to heat the material in the furnace. These electrodes may be raised in any well known manner (diagrammatic means only being indicated in the drawing) as the material in the furnace becomes fused. The powdered or broken carbonaceous material 3 may be covered with any suitable material 6, such as lime dust, to exclude the air therefrom.

I charge the floor of the furnace with lime, preferably pure calcium oxide and carbonaceous material, the charge as a whole being designated by numeral 7, the latter preferably being petroleum coke because it leaves substantially no ash. A substantial excess of coke beyond that required to react with the lime to form calcium carbide is used, and this material is placed on top of the charge on the furnace floor, filling the furnace as high as is desirable. When the arcs are struck, the temperature rises and calcium carbide forms and flows over the bottom 2 of the furnace, for calcium carbide is relatively thin at high temperatures. This fusion of the calcium carbide will tend to dissolve additional carbon.

As the temperature is raised the carbide at the bottom of the furnace is broken up, the calcium rising and perhaps forming more carbide with the carbonaceous material above, thus melting and fusing and perhaps dissolving more carbon until the reaction has worked progressively and entirely throughout the contents of the furnace. After all of the carbonaceous material has either been formed in the carbide or dissolved by the carbide and after the calcium has been driven off, the remaining slab or ingot is one of relatively dense graphite.

It will thus be seen that the reaction is carried out in zones progressively upward in the furnace, the graphite slab being the hottest zone and above it a layer of carbide becoming rich in graphite. Above this, the calcium vapor, driven off from the hot carbide reacts with carbonaceous material forming new carbide. The charge above these zones is heated by the ascending vapors and heat from the reactions below.

The member 4 is moved upward at the

same rate as the electrodes, so that it is not in the hottest zone. As the ingot forms upon the bottom 2 of the furnace, it is retained by the powdered carbon side walls 5 3 and this is advantageous as will appear hereinafter.

For some purposes a highly dense graphite is desirable and according to my process the density of the ingot so produced in the electric furnace may be increased due to its having 10 property similar to iron or other metals in that it can be mechanically worked to increase its specific gravity.

The design of furnace herein disclosed is 15 well adapted for cases when it is desired to compress the hot ingot. This may be done by transferring the entire furnace into a die and placing it in a press, or if the furnace wall and packing be strong enough for the 20 pressure desired, it can be used as the die itself and the pressure can be exerted directly upon the ingot from above.

It will thus be noticed that with the furnace herein disclosed the retaining receptacle 25 not only supports the lining and heat insulating material 3 but also excludes the air therefrom. Also the gases evolving from the reaction pass upwardly through the charge and not through the lining material.

Furthermore, it is to be understood that 30 the particular forms of apparatus shown and described, and the particular procedure set forth are presented for purposes of explanation and illustration and that various 35 modifications of said apparatus and procedure can be made without departing from my invention as defined in the appended claims.

What I claim is:

1. The process of making graphite which 40 consists in heating lime and carbonaceous material in a suitable furnace, whereby a fluid carbide is formed, and continuing the heating until the carbonaceous material has been transformed into graphite and the calcium volatilized.

2. The process of making relatively dense 50 graphite ingots which consists in placing carbonaceous material and a relatively small quantity of lime in a suitable furnace and heating until the carbonaceous material has been transformed in the presence of calcium to a relatively dense quality of graphite and the calcium volatilized.

55 3. The process of making relatively dense shapes of graphite which consists in heating in a suitable container of predetermined shape carbonaceous material and a flux capable of flowing the material and of breaking down upon continued heating into volatile matter and graphite.

4. The process of making relatively dense 60 shapes of graphite which consists in heating in a suitable container of predetermined shape a relatively large quantity of car-

bonaceous material and a relatively small quantity of material capable of combining with the carbonaceous material to flow it and upon continued heating capable of breaking down into volatile material and graphite. 70

5. The process of making relatively dense graphite ingots which consists in heating in an electric furnace a relatively large quantity of carbonaceous material and a relatively small quantity of lime until calcium carbide is formed and continuing the heating until all the calcium carbide is broken down into volatile material and graphite. 75

6. The process of making relatively dense ingots of graphite which consists in heating in an electric furnace a relatively large quantity of carbonaceous material and a relatively small quantity of lime until calcium carbide is formed and continuing the heating while the calcium is progressively volatilized, forming more carbide with the remaining carbonaceous material until the calcium is driven off leaving a relatively dense quantity of graphite. 80

7. The process of forming shapes of relatively dense graphite which consists in mechanically working relatively hot graphite. 85

8. The process of forming shapes of relatively dense graphite which consists in pressing relatively hot graphite in a die. 90

9. The process of forming relatively dense shapes of graphite which consists in mechanically working graphite while it is sufficiently hot to be plastic. 95

10. The process of making relatively dense shapes of graphite which consists in heating carbonaceous material with lime in an electric furnace until the calcium is volatilized, removing the graphite ingot and mechanically working it to increase its density. 100

11. The process of forming relatively dense shapes of graphite which consists in heating in an electric furnace carbonaceous material and a flux in a container of predetermined shape until the flux is volatilized, leaving a soft, hot graphite ingot, and mechanically pressing such ingot to increase its density and homogeneity. 105

12. The process of making relatively dense graphite shapes which consists in heating in an electric furnace carbonaceous material and lime until a relatively dense homogeneous ingot of graphite is produced, and mechanically working such ingot under pressure while it is hot and soft to produce a more dense and homogeneous shape of graphite. 115

13. The process of making relatively dense predetermined shapes of graphite which consists in heating in an electric furnace carbonaceous material and lime in a container of predetermined shape until a relatively dense homogeneous ingot of graphite is produced and mechanically working such ingot under pressure while it 120

- is hot and soft to produce a predetermined shape of graphite having increased density and homogeneity.
14. The process of increasing the density of graphite which consists in compressing relatively soft hot graphite.
15. The process of increasing the density of a slab of graphite which consists in heating such slab until it becomes relatively soft and compressing it.
16. The process of increasing the density and homogeneity of graphite which consists in heating it until it becomes plastic and applying a relatively great pressure thereto.
17. The process of increasing the density of carbonaceous material which consists in heating such material until it becomes soft and applying a relatively great pressure thereto.
18. The process of increasing the density of carbonaceous material which consists in heating such material in an electric furnace until it becomes plastic and applying a relatively high pressure thereto while it is confined in a relatively strong container.
19. The process of increasing the density of carbon which consists in heating it above a red heat and applying a pressure upon it while it is above a red heat.
20. The process of making graphite ingots which consists in forming a mold of relatively fine carbonaceous material and heating the carbonaceous material with a flux therein by means of an electric arc, whereby an ingot of graphite is cast in a pre-determined shape of the mold.
21. The process of forming relatively dense shapes of graphite which consists in forming a mold of lamp black of predetermined shape in a retaining member, placing a charge of carbonaceous material and flux inside a movable frame in said mold, heating the charge by means of an electric arc formed between movable electrodes and the floor of the mold, and simultaneously elevating the frame and electrodes.
22. An electric furnace for reacting on carbonaceous material comprising a retaining member, a lining of relatively fine carbonaceous material, a vertically movable frame to engage the sides of the lining and to receive the charge and vertically movable electrodes inside said frame to draw arcs from the bottom of the furnace.
23. An electric furnace construction comprising a trough-shaped retaining member, a lining for the sides and bottom of relatively fine carbonaceous material, a floor of carbon slabs upon the bottom of said lining, a movable frame engaging the sides of said lining, and superposed above said floor, said frame and floor forming a receptacle for the charge, and electrodes for drawing arcs through a portion of the charge.
- In testimony whereof, I hereunto affix my signature.

VICTOR M. WEAVER.